# EUROPEAN PATENT SPECIFICATION

(11) **EP 2 730 352 B1**
(45) Date of publication and mention of the grant of the patent: **01.08.2018**
(21) Application number: 13191615.7
(22) Date of filing: 05.11.2013
(51) Int. Cl.: B22D 41/30

(54) **MANUFACTURING METHOD OF RECYCLED PLATE FOR SLIDING NOZZLE**
HERSTELLUNGSVERFAHREN EINER WIEDERVERWENDETEN PLATTE FÜR EINE SCHIEBEDÜSE
PROCÉDÉ DE FABRICATION DE PLAQUE RECYCLÉE POUR BUSE COULISSANTE

(30) Priority: 12.11.2012 JP 2012248408
(43) Date of publication of application: 14.05.2014
(73) Proprietor: TYK Corporation, Tokyo 108-0075 (JP)
(72) Inventor: HATTANDA, Hirokatsu, Tajimi-shi, Gifu 507-8607 (JP)
(74) Representative: Epping - Hermann - Fischer

(56) References cited:
- DE-A1- 3 527 756
- GB-A- 2 060 842
- JP-A- H03 180 264
- JP-A- 2009 233 685

## Description

### Technical Field

The present invention relates to a manufacturing method of a recycled plate for a sliding nozzle, the method including performing processing for extending an endurance period on a plate used for the sliding nozzle that performs discharge control and flow control of molten steel in a steel manufacturing process.

### 2. Description of the Related Art

### Background Art

A sliding nozzle is a device that is used for discharge control and flow control of molten steel when discharging the molten steel from a molten steel vessel such as a ladle and a tundish in a steel manufacturing process. As illustrated in Fig. 6, a common sliding nozzle 110 includes two plates of a fixed plate 111 and a movable plate 112 that are formed by refractory bricks. The fixed plate 111 is fixed to the bottom portion of an upper nozzle 101 fitted into an opening of a bottom portion 90 of the molten steel vessel. The movable plate 112 is a plate that reciprocates or rotates while sliding relative to the fixed plate 111. A lower nozzle 102 is fixed to the movable plate 112. Holes 111h and 112h penetrate through the fixed plate 111 and the movable plate 112, respectively. The position of the hole 111h of the fixed plate 111 is identical to an opening 101p of the upper nozzle 101 and the position of the hole 112h of the movable plate 112 is identical to an opening 102p of the lower nozzle 102. With this configuration, if the movable plate 112 slides relative to the fixed plate 111, the opening 101p of the upper nozzle 101 and the opening 102p of the lower nozzle 102 are switched to be communicated or non-communicated with each other. This controls discharge or stop of the discharge of the molten steel from the molten steel vessel. Furthermore, the size of a space through which the opening 111h of the fixed plate 111 and the opening 112h of the movable plate 112 are communicated is changed so as to perform flow control of the molten steel.

Although the sliding nozzle 110 including two plates (the fixed plate 111 and the movable plate 112) is illustrated in Fig. 6, a sliding nozzle 120 including three plates of an upper fixed plate 121, a lower fixed plate 122, and a movable plate 123 has been used conventionally, as illustrated in Fig. 7. The upper fixed plate 121 is fixed to the upper nozzle 101 fixed to the bottom portion 90 of the molten steel vessel. The lower fixed plate 122 is unmovable and the lower nozzle 102 is attached to the lower fixed plate 122. The movable plate 123 slides between the upper fixed plate 121 and the lower fixed plate 122.

The plates used for the sliding nozzle as described above are severely damaged with use. For example, portions of the plates that make contact with the molten steel are eroded physically by the flowing molten steel. Furthermore, the temperature of the molten steel is extremely high, so that cracking is occurred on the plates due to thermal shock. The cracking is also occurred by structural spalling due to penetration of the molten steel into matrices of the plates. In addition, contents of a refractory material constituting the plates are lost because of elution into the molten steel or gasification, so that the matrices become porous. Moreover, the plates slide relatively, so that contact surfaces thereof are worn and the surface roughness is increased.

The endurance periods of the plates for the sliding nozzle used under such a severe environment are short and the plates need to be exchanged by brand-new plates, frequently. This arises a problem that the cost is increased. Furthermore, in order to avoid a significant trouble such as leakage of the molten steel, the plates are exchanged by the brand-new plates earlier than the usage limits thereof, resulting in waste of resources.

In order to solve the above problems, the present applicant has proposed a recycling method of performing processing for extending an endurance period on a used plate in the past (see, Japanese Patent No. 4980275). The recycling method is a method of impregnating a refractory layer of the used plate with tar or pitch, and then, heating it so as to remove a volatile component from the tar or the pitch.

With this method, the tar or the pitch penetrates into cracking, recesses on the surface having the increased roughness, and increased opening pores that are occurred on the refractory layer of the plate with use so as to densify the refractory layer. Further, extension of the cracking is suppressed with an adhesiveness of the tar or the pitch. Accordingly, the above-mentioned recycling method is capable of extending the endurance period of the used plate. Moreover, the recycled plate can be distributed at lower cost than a brand-new product. This makes it possible to reduce the cost taken for maintaining the sliding nozzle and use resources effectively.

However, with the above-mentioned conventional method, when the recesses such as the cracking occurred on the plate with use are minute, the recesses can be repaired with the impregnation of the tar or the pitch but the recesses having large sizes at some degree cannot be repaired. For this reason, the used plate on which even less recesses having the large sizes have been occurred cannot be recycled with the above-mentioned method. In consideration of this, a technique that makes it possible to recycle even a plate on which recesses having large sizes have been occurred and widen a range of the used plate as a target for recycling has been required.

### Summary of Invention

### Technical Problem

In view of the above-mentioned circumstances, an object of the invention is to provide a manufacturing method of a recycled plate, which is capable of repairing damage of a plate used for a sliding nozzle to extend an endurance period and widens a range of the used plate as a target for recycling.

### Solution to Problem

In order to solve the above-mentioned problem, a manufacturing method of a recycled plate for a sliding nozzle (hereinafter, simply referred to as "manufacturing method" in some cases) according to claim 1 is provided. Preferred embodiments are set forth in the subclaims.

The "plate for the sliding nozzle" may be a plate that is used by combining two plates of a fixed plate and a movable plate as described above, or a plate that is used by combining three plates of an upper fixed plate, a lower fixed plate, and a movable plate sliding between the upper fixed plate and the lower fixed plate. Further, the relative sliding direction of the plate may be any of reciprocation and rotation. That is to say, the aspect of the invention can be applied to an arbitrary plate that slides relatively to the other plate so as to communicate or non-communicate the respective through-holes.

As the "refractory brick", refractory bricks of high alumina based refractory, alumina-magnesia based refractory, magnesia based refractory, zirconia based refractory, alumina-carbon based refractory, magnesia-carbon based refractory, alumina-magnesia-carbon based refractory, alumina-spinel-carbon based refractory, and alumina-zirconia-carbon based refractory can be exemplified.

The carbon based refractory brick has advantages such as high resistance to thermal shock, low thermal expansion coefficient, excellent resistance to chemical erosion, and low wettability to molten steel. Therefore, the carbon based refractory brick is suitable as the refractory brick constituting the plate that is used under the severe environment. On the other hand, the carbon based refractory brick has a disadvantage that it is easy to be oxidized if being heated in the atmosphere because it is carbon based. In addition, a carbon content of the molten steel is extremely low, so that the carbon is easy to be eluted into the molten steel from the carbon based refractory brick due to contact with the molten steel in the steel manufacturing process. That is to say, the carbon content of the carbon based refractory brick is lost with oxidization reaction and elution. Therefore, it is difficult to prevent the matrix from becoming porous. Accordingly, the aspect of the invention in which the matrix of the refractory brick is impregnated with the liquid containing at least one of the tar and the pith is suitable particularly as a manufacturing method of a recycled product of the plate formed by the carbon based refractory brick of which matrix becomes porous with use inevitably.

As "the tar or the pitch", dehydrated tar, coal pitch, and petroleum pitch can be exemplified. Although the coal pitch is classified into soft pitch (softening temperature of equal to or lower than approximately 70°C), middle pitch (softening temperature of 70 to 85°C), and hard pitch (softening temperature of equal to or higher than approximately 85°C) based on the softening temperature, any of them can be used. Further, the liquid containing at least one of the tar and the pitch may be liquid containing at least only one of the tar and the pitch or may be liquid in which at least one of the tar and the pitch is diluted with a solvent. The pitch as a solid at a normal temperature is used in a state of being made into liquid by being heated to equal to or higher than the softening temperature or a state of being dissolved in a solvent.

The heating after the impregnation is performed in order to remove the volatile component contained in the tar and/or pitch impregnated into the matrix. Note that complete removable of the volatile component is not essential.

As the "thermal expandable refractory material of which volume is increased by generation reaction with heating", a refractory material containing a raw material with which ceramics having a lower density than the raw material is synthesized with heating can be used. Alternatively, a refractory material containing metallic powder with which metal oxide is generated by oxidization with heating can be used.

As the "thermal expandable refractory material of which volume is increased by change in a crystal structure with heating", a refractory material containing a ceramics material of which crystal structure is changed with heating to be transferred to a crystal phase having a lower density can be used.

With the manufacturing method, the tar and/or the pitch is made to penetrate into opening pores of the matrix that has become porous and brittle in the plate damaged with use. As a result, the opening pores are filled with the tar and/or the pitch and the matrix is densified. In addition, extension of cracking and enlargement of peeling are prevented with the adhesiveness of the tar or the pitch.

The impregnation of the tar and/or the pitch can be performed by immersing the entire plate into liquid for impregnation. This enables the damage of the plate to be repaired entirely. With this, the peripheral edge of the through-hole through which the molten steel is distributed, the surface of the plate that makes contact with the molten steel while the discharge of the molten steel is stopped, and the surface that is damaged due to relative sliding between the plates can be repaired simultaneously.

The peripheral edge of the through-hole of the plate is a portion that is damaged at the most significant level. As a reason of this, the peripheral edge of the through-hole of the plate is easy to be eroded physically by the molten steel flowing down the through-hole and cracking due to thermal shock is easy to be occurred thereon with contact with the molten steel at a high temperature. Therefore, there is a risk that the damage on the peripheral edge of the through-hole is not repaired sufficiently with the impregnation of the tar and/or the pitch only. In the manufacturing method, the peripheral edge of the through-hole is cut so as to remove the portion that has been damaged at the most significant level. With this, the inner wall of the through-hole becomes a new surface that is less damaged, so that resistance to the molten steel is restored.

In the manufacturing method, since the impregnation of the tar and/or the pitch is performed before the cutting of the peripheral edge of the through-hole, the matrix of the plate that has become porous and brittle with use is densified. This makes it possible to perform mechanical cutting easily and cut the peripheral edge of the through-hole well.

When the recess occurred on the plate surface due to cracking, peeling, or the like is minute, the recess is filled by the impregnation of the tar and/or the pitch. However, when the opening width and the depth of the recess are large at some degree, the recess is not filled sufficiently by the impregnation of the tar and/or the pitch only. In order to cope with this, in the aspect of the invention, even the recess having such size that is not filled with the tar and/or the pitch sufficiently is filled with the thermal expandable refractory material. The thermal expandable refractory material filled into the recess is heated under a high-temperature environment when the plate is reused so as to thermally expand. That is to say, the recess is filled with the material that does not shrink thermally at a high temperature unlike common mortar, so that a state where the recess is filled is maintained long. Accordingly, a recycled plate of which endurance period is extended long can be manufactured with the manufacturing method.

Further, the manufacturing method makes it possible to recycle a used plate with the recess having such size that is not filled with the tar and/or the pitch, thereby a range of the used plate as a target for recycling is widened.

The size of the recess into which the thermal expandable refractory material is filled is set to "an opening width and a depth of equal to or smaller than 1 mm" for the following reason. That is, there arises a risk that filling into the recess having the opening width and the depth of larger than 1.0 mm with the thermal expandable refractory material becomes insufficient.

In the manufacturing method of the recycled plate for the sliding nozzle according to the aspect of the invention, it is preferable that "the recycling processing further include grinding a surface of the plate before the recess is filled with the thermal expandable refractory material after the plate has been impregnated with the liquid and heated, and bonding a plate material to one surface of the plate after having been grinded."

The grinding is performed after the impregnation and the heating and before the filling of the thermal expandable refractory material, and can be performed before or after the cutting of the peripheral edge of the through-hole. Further, the bonding of the plate material, which is performed after the grinding, is not needed to be performed immediately after the grinding. For example, the bonding of the plate material can be performed after the filling of the thermal expandable refractory material.

When the recess occurred on the plate due to cracking, peeling, or the like is minute, the recess is filled by the impregnation of the tar and/or the pitch. However, when the opening width and the depth of the recess are large at some degree, the recess is not filled sufficiently by the impregnation of the tar and/or the pitch only. For coping with this, in the aspect of the invention, the surface of the plate after the impregnation and the heating is grinded. For example, the grinding is performed such that the surface of the plate is removed by 0.5 mm to 1.0 mm. Since the impregnation is performed before the grinding, the matrix of the plate that has become porous and brittle with use is densified. This makes it possible to perform mechanical grinding easily and suppress peeling of the plate surface with the grinding.

The grinding makes the plate surface smooth and reduce the number of recesses having such large sizes that have not been filled with the tar and/or the pitch by the impregnation. Further, the recess that remains after the grinding becomes shallower than that before the grinding. Therefore, in the filling of the thermal expandable refractory material, which is to be performed subsequently, the recess is filled sufficiently. Accordingly, since the grinding is performed after the impregnation and before the filling in the recycling processing, the used plate with the recess having such size that cannot be repaired with the conventional technique can be recycled, thereby a range of the used plate as a target for recycling is widened. It is to be noted that the grinding may be performed on one surface of the plate or both surfaces thereof.

In addition, in the manufacturing method, the thickness of the plate which has become thinner than the original thickness by the grinding is adjusted by a plate material. The thickness of the plate material to be bonded is set desirably such that the thickness of the plate to which the plate material has been bonded after the grinding is equal to the thickness of the plate before the grinding in a state where the plate is attached to the sliding nozzle to be used. With this, the recycled plate can be attached to the sliding nozzle to be used without requiring the sliding nozzle to perform any adjustment. It is to be noted that a plate material made of a metal or ceramics can be used for the plate material. Further, the plate material is bonded to the surface opposite to the surface of the plate that slides relatively to the other plate.

In the manufacturing method of the recycled plate for the sliding nozzle according to the aspect of the invention, it is preferable that "the plate on which the recycling processing has been performed be attached to the sliding nozzle, be used, and then, be detached from the sliding nozzle, and the recycling processing be performed on the plate, again".

Conventionally, the plate is reused once at most. On the other hand, with the aspect of the invention in which the impregnation of at least the tar and/or the pitch, the cutting of the peripheral edge of the through-hole, and the filling of the thermal expandable refractory material are performed, the plate that has been damaged with use is repaired at the high degree. With this, the above-mentioned configuration in which the recycled plate is attached to the sliding nozzle, is used, and then, the recycling processing is further performed thereon so as to obtain the recycled plate again can be employed.

Accordingly, with the manufacturing method, the endurance period of one plate is made longer. As a result, the cost for operating the sliding nozzle can be further reduced, thereby resources can be utilized more effectively.

### Effects of Invention

As described above, as an effect of the invention, a manufacturing method of a recycled plate, which is capable of repairing damage of a plate used for a sliding nozzle to extend an endurance period and widens a range of the used plate as a target for recycling, can be provided.

### Brief Description of Drawings

Fig. 1 is a flowchart of recycling processing in a manufacturing method according to a first embodiment.
Fig. 2 is a flowchart of recycling processing in a manufacturing method according to a second embodiment.
Fig. 3 is a cross-sectional view in a state where a recycled plate is attached to a sliding nozzle.
Fig. 4 is a flowchart of a manufacturing method in which the recycling processing is performed once.
Fig. 5 is a flowchart of a manufacturing method in which the recycling processing is performed twice.
Fig. 6 is a cross-sectional view illustrating a common sliding nozzle including two plates.
Fig. 7 is a cross-sectional view illustrating a common sliding nozzle including three plates.

### Description of Embodiments

Hereinafter, described are specific embodiments of the invention with reference to Fig. 1 to Fig. 5. In any of manufacturing methods according to a first embodiment and a second embodiment, a used plate is detached from a sliding nozzle, recycling processing PI is performed on the used plate, and a manufactured recycled plate is attached to the sliding nozzle, is used again, as illustrated in Fig. 4.

The recycling processing PI in the manufacturing method according to the first embodiment is performed in the order of impregnation S1, heating S2, blasting S3, hole edge cutting S4, and filling S5 as the flow thereof is illustrated in Fig. 1.

### Impregnation S1:

A used plate is immersed in liquid containing at least one of tar and pitch so as to impregnate a matrix of the plate with the liquid. The viscosity of the liquid for impregnation is changed by heating or diluting the liquid so as to adjust the easiness of penetration of the liquid into the matrix. If opening pores of the matrix are deaerated while the used plate is placed at a reduced pressure before the impregnation, the matrix is impregnated with the liquid effectively. A larger amount of liquid can be made to penetrate into the matrix forcibly by impregnating the matrix with the liquid while pressurizing the liquid.

Contents of the matrix of the used plate are lost because of elution into molten steel or gasification, so that the opening pores are increased. The liquid containing the tar and/or the pitch penetrates into the opening pores and a layer of the tar and/or the pitch is formed. Further, recesses such as cracking and peeling traces are formed on the surface of the plate and the tar and/or the pitch is also filled into the minute recesses.

### Heating S2:

Heating conditions are set to 200°C to 400°C (baking) and 500°C to 700°C (caulking). Heating removes a volatile component from the tar and/or the pitch impregnated into the matrix of the plate. This prevents smoking from the plate while the plate is used by being attached to the sliding nozzle.

### Blasting S3:

Residues of the tar and/or the pitch remain on the surface of the plate after heated. Then, blasting particles (projection materials) are blasted onto the surface of the plate so as to remove the residues. The conditions such as a type, a particle diameter, and a blasting speed of the blasting particles can be set appropriately in accordance with the type of the refractory brick constituting the plate, the type of the tar and/or the pitch, and the like.

### Hole Edge Cutting S4

A peripheral edge of a through-hole on the used plate is cut by a cutting tool. The through hole of the common plate has a circular cross-sectional shape and is cut concentrically. Since the impregnation S1 is performed before the hole edge cutting S4, the matrix of the plate that has become porous and brittle with use is densified. This makes it possible to perform mechanical cutting easily and cut the peripheral edge of the through-hole well.

The peripheral edge of the through-hole on the plate is a portion that is damaged at the most significant level. As a reason of this, the peripheral edge of the through-hole of the plate is easy to be eroded physically by the molten steel flowing down the through-hole and cracking due to thermal shock is easy to be occurred thereon with contact with the molten steel at a high temperature. The peripheral edge of the through-hole is cut so as to remove a portion that has been damaged at the most significant level. With this, the inner wall of the through-hole becomes a new surface that is less damaged, so that resistance to the molten steel is restored.

Although the through-hole of the plate is enlarged by the hole edge cutting S4, the plate is used as a recycled plate while keeping the size of the through-hole. For example, there are common sliding nozzles of a plurality of types having different nozzle opening diameters of 60 mm, 65 mm, 70 mm, and the like. When the sliding nozzles of the plurality of types having the different nozzle opening diameters are used in the same facility, a plate used for the sliding nozzle having a smaller opening diameter is recycled and can be attached to the sliding nozzle having a larger opening diameter to be reused. Further, in the conventional plates that have been used in an overlapped manner, the diameters of through-holes thereof are made identical in normal cases. However, if the diameters of the through-holes of the plates are different, control of discharge and stop of the discharge of the molten steel and flow control can be performed with no special problem.

### Filling S5:

The recesses having the opening widths and the depths of equal to or smaller than 1 mm are filled with a thermal expandable refractory material of which volume is increased by at least one of generation reaction and change in a crystal structure with heating when the plate attached to the sliding nozzle is used. With this, the recesses that have not been sufficiently filled with the tar and/or the pitch in the impregnation S1 are filled with the thermal expandable refractory material. It is to be noted that the recesses having the opening widths and the depths of equal to or smaller than 0.01 mm have been filled with the tar and/or the pitch in the impregnation S1. Therefore, it is sufficient that the recesses having the opening widths and the depths of equal to or larger than 0.01 mm and equal to or smaller than 1 mm are filled with the thermal expandable refractory material.

As the thermal expandable refractory material, (1) a material obtained by kneading a refractory material containing raw materials with which ceramics having a lower density than the raw materials is synthesized with heating with a liquid medium (water, organic solvent), (2) a material obtained by kneading a refractory material containing metallic powder with which metal oxide is generated by oxidization with heating with the liquid medium (water, organic solvent), or (3) a material obtained by kneading a refractory material containing a ceramics material of which crystal structure is changed with heating to be transferred to a crystal phase having a lower density with the liquid medium (water, organic solvent) can be used.
(1) As the raw materials with which ceramics having a lower density than the raw materials is synthesized with heating, aluminum oxide and silicon dioxide with which mullite is synthesized with heating, magnesium oxide and aluminum oxide with which spinel is synthesized with heating, and titanium oxide and aluminum oxide with which aluminum titanate is synthesized with heating can be exemplified.

Then, described is the change in volume by the synthesis (generation reaction) of mullite. Molecular weights and densities of aluminum oxide (Al₂O₃), silicon dioxide (SiO₂), and mullite (3Al₂O₃●2SiO₂) are as follows:
Aluminum oxide: molecular weight 102, density 3.99 (as corundum)
Silicon dioxide: molecular weight 60, density 2.53 (as quartz)
Mullite: molecular weight 426, density 3.17

Accordingly, the volume after generation of 1 mol of mullite is increased in comparison with that before the generation as follows:
Volume before generation (3Al₂O₃ + 2SiO₂): 124.1 cm³
Volume after generation (3Al₂O₃●2SiO₂): 134.4 cm³

Described is the change in volume by synthesis (generation reaction) of spinel. Molecular weights and densities of magnesium oxide (MgO), aluminum oxide (Al₂O₃), and spinel (MgO•Al₂O₃) are as follows:
Magnesium oxide: molecular weight 40, density 3.65
Aluminum oxide: molecular weight 102, density 3.99 (as corundum)
Spinel: molecular weight 142, density 3.60

Accordingly, the volume after generation of 1 mol of spinel is increased in comparison with that before the generation as follows:
Volume before generation (MgO + Al₂O₃): 36.5cm³
Volume after generation (MgO●Al₂O₃): 39.4cm³

Described is the change in volume by synthesis (generation reaction) of aluminum titanate. Molecular weights and densities of titanium oxide (TiO), aluminum oxide (Al₂O₃), and aluminum titanate (TiO₂●Al₂O₃) are as follows:
Titanium oxide: molecular weight 80, density 4.25 (as rutile)
Aluminum oxide: molecular weight 102, density 3.99 (as corundum)
Aluminum titanate: molecular weight 182, density 3.65

Accordingly, the volume after generation of 1 mol of aluminum titanate is increased in comparison with that before the generation as follows:
Volume before generation (TiO₂ + Al₂O₃): 44.3 cm³
Volume after generation (TiO₂●Al₂O₃): 49.8 cm³

The metal oxides as the raw materials with which composite oxide ceramics having a lower density than the raw materials is synthesized with heating, such as aluminum oxide, silicon dioxide, magnesium oxide, and titanium oxide, have average particle diameters of 0.1 µm to 20 µm, and preferably 0.1 µm to 10 µm. If the metal oxides are fine particles having the average particle diameters in the above-mentioned range, composite oxide ceramics (mullite, spinel, aluminum titanate) is easy to be generated with heating. Therefore, an action of increasing the volume of the thermal expandable refractory material with heating is easy to be exhibited. It is to be noted that the particle diameter can be obtained as a diffraction scattering diameter by a laser diffraction scattering method.

The ratios of the aluminum oxide and the silicon dioxide as the raw materials for generating mullite are set to be ratios closer to the stoichiometric composition of mullite. With this, substantially the total volume of the aluminum oxide and the silicon dioxide are turned into mullite and the degree of the increase in the volume of the thermal expandable refractory material under heating can be made large. The degree of the increase in the volume of the thermal expandable refractory material under heating can be adjusted by shifting the ratios of the aluminum oxide and the silicon dioxide as the raw materials for generating mullite from the stoichiometric composition of mullite. The same holds true for ratios of the magnesium oxide and the aluminum oxide as the raw materials for generating spinel and ratios of the titanium oxide and the aluminum oxide as the raw materials for generating aluminum titanate.

As the thermal expandable refractory material with which mullite is synthesized with heating, for example, a material obtained by kneading the refractory material having the following composition with water or an organic solvent can be exemplified:
Al₂O₃ (average particle diameter: 5 µm) 71 mass%
SiO₂ (average particle diameter: 1 µm) 24 mass%
Other contents (binder and the like) 5 mass%

As the thermal expandable refractory material with which spinel is synthesized with heating, a material obtained by kneading the refractory material having the following composition with water or an organic solvent can be exemplified. It is to be noted that the following composition is an example of the thermal expandable refractory material of which degree of thermal expansion is suppressed by lowering the ratio of magnesium oxide.
MgO (average particle diameter: 20 µm) 5 mass%
Al₂O₃ (average particle diameter: 5 µm) 92 mass%
Other contents (binder and the like) 3 mass%

The conventional refractory mortar that is used for bonding refractory bricks and forms a joint portion is obtained by mixing the refractory material and clay or a liquid glass as a binder (plasticizer) and kneading the mixed material with water generally. As the refractory material, aluminum oxide, silicon dioxide, and magnesium oxide are used in addition to dolomite, mullite, spinel, and the like in some cases. However, the powder of the refractory material for the conventional refractory mortar has a course average particle diameter as much as equal to larger than 70 µm. Therefore, even when aluminum oxide and silicon dioxide are contained at ratios overlapping with the above-mentioned composition, mullite is not generated with heating. Further, even when magnesium oxide and aluminum oxide are contained at ratios overlapping with the above-mentioned composition, spinel is not generated with heating.
(2) As the refractory material containing metallic powder with which metal oxide is generated by oxidization with heating, a refractory material containing powder of aluminum and a refractory material containing powder of iron can be exemplified. Further, the refractory material can contain aluminum oxide, mullite, spinel, or the like in addition to the metallic powder. The metallic powder reacts with water to generate heat and generate hydrogen gas. Therefore, the refractory material containing the metallic powder is used by being kneaded with an organic solvent or a liquid medium containing an organic solvent at a high ratio desirably.
(3) As the refractory material containing a ceramics material of which crystal structure is changed with heating to be transferred to a crystal phase having a lower density, a refractory material containing fine quartz powder is used. Cristobalite is precipitated from the fine quartz with heating. The cristobalite transforms to the α-cristobalite from the β-cristobalite at approximately 230°C and the volume thereof is increased.

After the recesses have been filled with the thermal expandable refractory material, the plate is heated at the temperature of 100°C to 300°C so as to dry the thermal expandable refractory material.

Next, described is the manufacturing method according to the second embodiment. In recycling processing P1 in the second embodiment, grinding S6 of the plate surface is further performed in addition to the recycling processing P1 in the first embodiment. The grinding S6 can be performed before or after the hole edge cutting S4. That is to say, the recycling processing P1 in the manufacturing method according to the second embodiment may be performed in the order of the impregnation S1, the heating S2, the blasting S3, the hole edge cutting S4, the grinding S6, and the filling S5 or in the order of the impregnation S1, the heating S2, the blasting S3, the grinding S6, the hole edge cutting S4, and the filling S5, as illustrated in Fig. 2. In the former case, bonding of the plate material that is performed after the grinding S6 can be performed before or after the filling S5. In the latter case, bonding of the plate material that is performed after the grinding S6 can be performed before or after the hole edge cutting S4 or after the filling S5.

### Grinding S6:

The plate surface is grinded by a grinder. For example, a grinder including a disc-like grinding stone is used and the plate surface is grinded by moving the grinder in parallel with the plate surface while rotating the grinding stone around an axis perpendicular to a plane of the plate. In this case, the grinding can be performed such that the surface of the plate is removed by 0.5 mm to 1.0 mm. Since the impregnation S1 is performed before the grinding S6, the matrix of the plate that has become porous and brittle with use is densified. This makes it possible to perform mechanical grinding easily and suppress peeling of the plate surface with the grinding.

The grinding S6 makes the plate surface smooth and reduce the number of recesses that have not been filled with the tar and/or the pitch in the impregnation S1. Further, the recesses that remain after the grinding S6 become shallower than that before the grinding S6. Therefore, in the filling S5 that is to be performed subsequently, the recesses are filled with the refractory material sufficiently.

In particular, the surface of the plate surfaces at the side that slides relatively to the other plate is damaged largely because the surface is rubbed while receiving a load. Since the lower plate of the rubbed two plates is kept making contact with the molten steel while the discharge of the molten steel is stopped, the lower plate is damaged largely. Therefore, it is effective to perform the grinding S6 on at least the surface of the plate surfaces at the side that slides relatively to the other plate.

The plate is made thinner than the original thickness by the grinding S6. Then, a plate material is bonded to the surface opposite to the surface of the plate that slides relatively to the other plate so as to adjust the thickness. In order to prevent the molten steel from being leaked from the contact surface with the other plate to which the plate slides relatively, large pressures are applied to the plate attached to the sliding nozzle from the upper and lower sides. For example, the pressure of 40 kN to 100 kN is applied by a spring member energizing such that frame members supporting the respective overlapped plates at the upper side and the lower side pressurize each other. Accordingly, the thickness of the plate material to be bonded to the plate after the grinding is set desirably such that the thickness of the plate to which the plate material has been bonded is equal to the thickness of the original plate in a state where the plate is attached to the sliding nozzle and the pressure is applied to the plate and the other plate from the upper and lower sides. If the thickness of the recycled plate in a state of being used is set to the thickness of the original plate in this manner, an additional member for adjustment for abutting two plates that are made to slide relatively is not required when the recycled plate is attached to the sliding nozzle to be used.

As described above, with the manufacturing method according to the second embodiment, the recycling processing P1 includes the grinding S6 in addition to the hole edge cutting S4 and the filling S5. This makes it possible to recycle a used plate that has been damaged largely, thereby a range of the used plate as a target for recycling is widened.

The recycled plate manufactured by the manufacturing method according to the first embodiment or the second embodiment can be reused by being attached to the sliding nozzle. The recycled plate attached to the sliding nozzle is heated under a high-temperature environment when used and the thermal expandable refractory material filled into the recesses expand. Thus, the recesses are filled with a material that does not shrink with heating, so that the state where the plate is repaired is maintained long. This makes it possible to extend the endurance period of the plate longer than that in the conventional technique.

The recycled plate manufactured by the manufacturing method according to the second embodiment is attached to the sliding nozzle as follows. That is, as illustrated in Fig. 3, a recycled plate 1 is attached to the sliding nozzle such that a surface 11 thereof opposite to a surface 12 bonded with a plate material 19 corresponds to the surface that slides relatively to the other plate 2. Fig. 3 illustrates a state where the recycled plate 1 is attached to an upper nozzle 40 and the brand-new plate 2 is attached to a lower nozzle 50.

As described above, with the manufacturing method according to the first embodiment or the second embodiment, even the plate having such large damage that cannot have been repaired conventionally can be recycled by performing the impregnation S1, the hole edge cutting S4, and the filling S5. This widens a range of the used plate as a target for recycling in comparison with the conventional technique.

Further, the degree that the plate damaged with use is repaired is higher in comparison with the conventional technique. This makes it possible to employ a manufacturing method in which the recycling processing of recycling a used plate to the recycled plate is performed a plurality of times. For example, as illustrated in Fig. 5, the following manufacturing method can be employed. That is, a plate is detached from a sliding nozzle, and a recycled plate subjected to the first recycling processing PI is attached to the sliding nozzle to be used. After using, the recycled plate is detached and second recycling processing P2 is performed thereon to obtain a recycled plate.

In the manufacturing method, the second recycling processing P2 can be performed in the same manner as the above-mentioned recycling processing P1. That is to say, the recycling processing P2 (S1-S2-S3-S4-S5) same as the recycling processing P1 in the manufacturing method according to the first embodiment and the recycling processing P2 (S1-S2-S3-S4-S6-S5 or S1-S2-S3-S6-S4-S5) same as the recycling processing PI in the manufacturing method according to the second embodiment can be performed. The above recycling processing PI and the recycling processing P2 can be combined appropriately.

As described above, the invention has been described by taking preferable embodiments as examples. However, the invention is not limited to the above-mentioned embodiments and various improvements and changes in design can be made in a range without departing from a scope of the invention as follows.

For example, the manufacturing method of performing the recycling processing once and the manufacturing method of performing the recycling processing twice have been described above. However, the invention is not limited thereto and the invention can be applied to a manufacturing method of performing the recycling processing equal to or more than three times.

The recycled plate manufactured by the manufacturing method according to the invention can be used by combining with another recycled plate or by combining with a brand-new plate.

### Reference Signs List

S1 IMPREGNATION
S2 HEATING
S3 BLASTING
S4 HOLE EDGE CUTTING
S5 FILLING
S6 GRINDING

### Citation List

### Patent Document

[Patent Document 1] Japanese Patent No. 4980275

## Claims

1. A manufacturing method of a recycled plate (1) for a sliding nozzle, the method comprising performing, on a plate after having been used for the sliding nozzle, recycling processing including:
impregnating a matrix of the plate that is formed by a refractory brick and has a through-hole with liquid containing at least one of tar and pitch;
heating the plate impregnated with the liquid to a baking temperature of 200°C to 400°C and a caulking temperature of 500°C to 700°C to remove a volatile component;
cutting a peripheral edge of the through-hole of the plate after having been impregnated with the liquid and heated, and
filling a recess having an opening width and a depth of equal to or smaller than 1 mm, which is present on a surface (11) of the plate having the through-hole of which peripheral edge has been cut, with a thermal expandable refractory material of which volume is increased by at least one of generation reaction and change in a crystal structure with heating when the plate attached to the sliding nozzle that performs discharge control and flow control of molten steel in a steel manufacturing process is used,
wherein the thermal expandable refractory material is selected from the group consisting of: a first material obtained by kneading a refractory material containing raw materials with which ceramics having a lower density than the raw materials is synthesized with heating with a liquid medium comprising water or organic solvent, wherein the raw materials comprise metal oxides having average particle diameters of 0.1 µm to 20 µm obtained as a diffraction scattering diameter by a laser diffraction scattering method, a second material obtained by kneading a refractory material containing metallic powder with which metal oxide is generated by oxidization with heating with the liquid medium, and a third material obtained by kneading a refractory material containing fine quartz powder with the liquid medium, wherein cristobalite is precipitated from the fine quartz and cristobalite transformation accompanied by a volume increase occurs with heating.

2. The manufacturing method of the recycled plate for the sliding nozzle according to claim 1, wherein
the recycling processing further includes:
grinding the surface (11) of the plate before the recess is filled with the thermal expandable refractory material after the plate has been impregnated with the liquid and heated, and
bonding a plate material (19) to the other surface (12) of the plate after having been grinded.

3. The manufacturing method of the recycled plate for the sliding nozzle according to claim 1 or 2, wherein
the plate on which the recycling processing has been performed is attached to the sliding nozzle , is used, and then, is detached from the sliding nozzle, and the recycling processing is performed on the plate, again.

## Patentansprüche

1. Herstellungsverfahren für eine wiederverwertete Platte (1) für eine Schiebedüse, wobei das Verfahren an einer Platte, die für die Schiebedüse benutzt wurde, ein Durchführen einer Wiederverwertungsverarbeitung umfasst, enthaltend:
Imprägnieren einer Matrix der Platte, die aus einem feuerfesten Ziegel ausgebildet ist und ein Durchgangsloch aufweist, mit einer Flüssigkeit, die mindestens eins aus Teer oder Pech enthält;
Erwärmen der mit der Flüssigkeit imprägnierten Platte auf eine Einbrenntemperatur von 200 °C bis 400 °C und eine Abdichttemperatur von 500 °C bis 700 °C, um einen flüchtigen Bestandteil zu entfernen;
Beschneiden einer umlaufenden Kante des Durchgangslochs der Platte, nachdem sie mit der Flüssigkeit imprägniert und erwärmt wurde, und
Füllen einer Vertiefung mit einer Öffnungsweite und einer Tiefe von gleich oder kleiner als 1 mm, die auf einer Fläche (11) der Platte vorhanden ist, die das Durchgangsloch aufweist, dessen umlaufende Kante beschnitten wurde, mit einem wärmeausdehnbaren feuerfesten Ziegelmaterial, dessen Volumen sich durch mindestens eins aus einer Bildungsreaktion und einer Änderung der Kristallstruktur beim Erwärmen vergrößert, wenn die an der Schiebedüse, die eine Austrittssteuerung und Durchflusssteuerung von Stahlschmelze in einem Stahlerzeugungsverfahren durchführt, angebrachte Platte benutzt wird,
wobei das wärmeausdehnbare feuerfeste Ziegelmaterial gewählt ist aus einer Gruppe, bestehend aus: einem ersten Material, erhalten durch ein Kneten eines feuerfesten Ziegelmaterials, das Rohstoffe enthält, mit denen eine Keramik mit einer geringeren Dichte als die Rohstoffe durch ein Erwärmen mit einem flüssigen Medium synthetisiert wird, das Wasser oder ein organisches Lösungsmittel umfasst, wobei die Rohstoffe Metalloxide mit mittleren Korndurchmessern von 0,1 µm bis 20 µm umfassen, erhalten als ein Beugungs-und Streuungsdurchmesser mit einem Laser-Beugungs- und - Streuungsverfahren, einem zweiten Material, erhalten durch ein Kneten eines Metallpulver, mit dem Metalloxid durch ein Erwärmen erzeugt wird, enthaltenden feuerfesten Ziegelmaterials mit dem flüssigen Medium, und einem dritten Material, erhalten durch ein Kneten eines feines Quarzpulver enthaltenden feuerfesten Ziegelmaterials mit dem flüssigen Medium, wobei Cristobalit aus dem feinen Quarzpulver gefällt wird und eine von einer Volumenerhöhung begleitete Cristobalitumformung beim Erwärmen auftritt.

2. Herstellungsverfahren für die wiederverwertete Platte für die Schiebedüse nach Anspruch 1, wobei
die Wiederverwertungsverarbeitung weiter enthält:
Schleifen der Fläche (11) der Platte, bevor die Vertiefung mit dem wärmeausdehnbaren feuerfesten Ziegelmaterial gefüllt wird, nachdem die Platte mit der Flüssigkeit imprägniert und erwärmt wurde, und
Kleben eines Plattenmaterials (19) auf die andere Fläche (12) der Platte, nachdem sie geschliffen wurde.

3. Herstellungsverfahren für die wiederverwertete Platte für die Schiebedüse nach Anspruch 1 oder 2, wobei
die Platte, an der die Wiederverwertungsverarbeitung durchgeführt wurde, an der Schiebedüse angebracht wird, benutzt wird und dann von der Schiebedüse abgenommen wird und wieder die Wiederverwertungsverarbeitung an der Platte durchgeführt wird.

## Revendications

1. Méthode pour fabriquer une plaque recyclée (1) pour une busette coulissante, la méthode comprenant l'exécution, sur une plaque après qu'elle ait été utilisée pour la busette coulissante, d'un traitement de recyclage comprenant :
imprégner une matrice sur la plaque qui est formée par une brique réfractaire et possède trou débouchant avec un liquide contenant au moins l'un du goudron et du brai ;
chauffer la plaque imprégnée avec le liquide à une température de cuisson de 200°C à 400°C et une température de calfeutrage de 500°C à 700°C afin d'éliminer un composant volatile ;
couper un bord périphérique du trou débouchant de la plaque après qu'elle ait été imprégnée avec le liquide et chauffée, et
remplir un retrait présentant une largeur d'ouverture et une profondeur égales ou inférieures à 1 mm, qui est présent sur une surface (11) de la plaque comportant le trou débouchant dont le bord périphérique a été coupée, d'une matière réfractaire thermiquement dilatable dont le volume est accru par au moins l'un d'une réaction de génération et d'un changement dans une structure cristalline avec chauffage lorsqu'est utilisée la plaque fixée sur la busette coulissante qui exécute le contrôle de décharge et le contrôle de débit d'acier fondu dans un processus de fabrication d'acier,
dans laquelle la matière réfractaire thermiquement dilatable est sélectionnée dans le groupe composé de : une première matière obtenue par pétrissage d'une matière réfractaire contenant des matières brutes avec lesquelles est synthétisée une matière céramique présentant une densité inférieure à celle des matières brutes, avec chauffage avec un milieu liquide contenant de l'eau ou un solvant organique, dans laquelle les matières brutes contiennent des oxydes métalliques possédant des diamètres de particules moyen de 0,1 µm à 20 µm obtenus en tant que diamètre de dispersion diffractive par une méthode de dispersion diffractive au laser, une seconde matière obtenue par pétrissage d'une matière réfractaire contenant une poudre métallique avec laquelle est généré un oxyde métallique par oxydation, avec chauffage avec le milieu liquide, et une troisième matière obtenue par pétrissage d'une matière réfractaire contenant une fine poudre de quartz avec le milieu liquide, dans laquelle la cristobalite est précipitée depuis le quartz fin et la transformation de cristobalite, accompagné d'une augmentation de volume apparaissant durant le chauffage.

2. Méthode pour fabriquer la plaque recyclée pour la busette coulissante selon la revendication 1, dans laquelle
le traitement de recyclage comprend en outre :
meuler la surface (11) de la plaque avant que le retrait soit rempli avec la matière réfractaire thermiquement dilatable après que la plaque ait été imprégnée avec le liquide et chauffée, et
lier une matière de plaque (19) sur l'autre surface (12) de la plaque après qu'elle ait été meulée.

3. Méthode pour fabriquer la plaque recyclée pour la busette coulissante selon la revendication 1 ou 2, dans laquelle
la plaque sur laquelle a été exécutée le traitement de recyclage est fixée sur la busette coulissante, utilisée, puis détachée de la busette coulissante, et le traitement de recyclage est à nouveau exécuté sur la plaque.
